

Nov. 24, 1953

**C. B. FOSTER**

2,660,525

## METHOD OF EXTRACTING LEAD FROM ITS SULFIDES

Filed Jan. 22, 1952

3 Sheets-Sheet 1



Fig. 2.



Fig. 3.

INVENTOR.  
CHARLES B. FOSTER  
BY

Townsend and Townsend  
ATTORNEYS

Nov. 24, 1953

C. B. FOSTER

2,660,525

METHOD OF EXTRACTING LEAD FROM ITS SULFIDES.

Filed Jan. 22, 1952

3 Sheets-Sheet 2



INVENTOR.

CHARLES B. FOSTER  
BY

Townsend and Townsend  
ATTORNEYS

Nov. 24, 1953

C. B. FOSTER

2,660,525

## METHOD OF EXTRACTING LEAD FROM ITS SULFIDES

Filed Jan. 22, 1952

3 Sheets-Sheet 3



*INVENTOR.*  
*CHARLES B. FOSTER*

. BY

Townsend and Townsend  
ATTORNEYS.



and because of inaccurate mechanical means so far developed to control the chemical reaction, successful operation of the plant is considerably dependent upon the personal skill and judgment of its operators.

In the instant invention I have provided a method wherein the chemical reaction as above set forth, takes place entirely within a closed circuit, wherein all dust, fumes, and gases are captured without the possibility of any of them escaping from without the enclosure into the open air. Thus, not only have I greatly minimized the risk and danger of lead poisoning for personnel working within the neighborhood of the plant, but I have also provided a means whereby the costly dust and silver loss is reduced to a minimum. Furthermore, because I am able to mechanically control with great accuracy the chemical reactions taking place in the process, I am not so dependent upon the personal skill and judgment of the plant operator as is the case in operating a Scotch hearth.

Although recovery in a blast furnace is the most commonly employed means of extracting lead from its ores, there are inherently multiple disadvantages attendant in employing this system, which my invention as presently described will entirely abrogate or greatly minimize.

In conventional and current lead-blast furnace practice, a quantity of the ore, Galena, is roasted at a reduced heat in the sintering plant. This process is not only costly, but results in a considerable dust loss. Furthermore, the actual sulfide of the ore combines with the oxygen in the air to form primarily lead oxide (PbO) and sulphur dioxide (SO<sub>2</sub>) along with smaller amounts of lead sulphate (PbSO<sub>4</sub>). Thus, the elimination of the sulphur existing in the form of a sulfide during sintering wastes the natural reducing power and calorific power of the Galena, thus making necessary the later use of carbon in some form to serve as a reducing agent and also as a fuel during the actual smelting of the ore in the blast furnace at a high temperature.

The extreme fineness of present day high-grade ore concentrate is not suited for use in a blast furnace because of increased dust loss as well as clogging of the blast furnace when such finely-divided concentrate is subjected to the air blast in the furnace. One of the objects in sintering the ore is to provide a coarse, porous product suitable for use within the blast furnace.

Although currently available lead ore concentrates are very high-grade, it has been found economically and practically expedient to excessively dilute this concentrate before considering it suitable for introduction into a blast furnace.

Furthermore, the sulphur dioxide gas which is evolved at the sintering plant is so highly diluted with surplus air that even after removal of dust and volatile impurities it is not generally considered commercially feasible to utilize this gas in acid manufacture.

Further disadvantages attendant with blast furnace operations are that the initial installation involves a large capital investment generally contemplating additional detached plants for the manufacture of intermediate and by-products, and also the fact that the starting and shutting down of blast furnaces is costly and results in a considerable time loss.

The instant invention is designed specifically to overcome these objections applicable to blast furnace operation. For example, sintering the

ore is both unnecessary and undesirable in practicing my method. Therefore, the natural reducing and calorific power of the sulfide ore is not lost by sintering, but is fully preserved and utilized to the utmost extent as hereinabove pointed out. Furthermore, the fineness of present day ore concentrate is especially suited for use in my process as the more finely divided the particles of ore, the more readily and completely will they react with the molten lead oxide. Again, the current high-grade ore concentrate may be employed without dilution in practicing my process, and furthermore the relatively undiluted sulphur dioxide gas which is given off during the reaction may be subsequently recovered for suitable acid manufacture. It should also be pointed out that both the initial installation cost and the cost of starting and stopping my apparatus is much less than the installation and/or operating cost for a conventional type blast furnace.

A principal object of this invention is to provide a new and practical method of lead reduction which utilizes to great advantage currently available, relatively high-grade quality, lead ore concentrates in the reduction process without the necessity of excessively diluting the said concentrates.

Another object of this invention is to provide a continuous, thermally self-sustaining method of metal reduction which requires no application of external heat to accomplish the reduction of metal from its concentrate after operations have been commenced, as will more fully appear hereinafter.

Another object of my invention is to provide a method which utilizes the natural self-contained calorific properties and the natural reducing power of simple sulfide ore concentrates to accomplish the reduction of metal therefrom.

Another object of this invention is to provide a method which takes full advantage of currently available, high-grade sulfide ore concentrates by introducing them into a reaction chamber without expensive dust loss and/or without the necessity of providing for large and expensive installations for dust recovery.

Another object of the invention is to provide a method which may be practiced in an apparatus which is relatively inexpensive to install and to operate as compared to cost of installation and operation of known types of apparatus in more or less common usage today, as above mentioned.

Another object of my invention is to produce as a by-product a highly concentrated sulphur dioxide gas suitable for acid manufacture.

Further objects of my invention will become apparent upon the reading of the specification and referring to the accompanying drawings in which similar characters of reference represent corresponding parts in each of the several views.

In the drawings:

Fig. 1 is a schematic view of a suitable apparatus in which the process may be practiced.

Fig. 2 is a sectional view taken on line 2-2 of Fig. 1.

Fig. 3 is an enlarged perspective view of the impellor incorporated in the apparatus.

Fig. 4 is a top plan view of a preferred embodiment of the apparatus.

Fig. 5 is a sectional view taken on line 5-5 of Fig. 4.

Fig. 6 is a sectional view taken on line 6-6 of Fig. 4.

75 In accordance with the present invention I

accomplish the conversion of a lead sulfide to the free metal and sulphur dioxide in two separate steps. The first of these steps is an oxidation step wherein the metal in molten condition is reacted in an oxidation zone with molecular oxygen to convert a portion thereof to the oxide in accordance with the following general reaction:



The second or reduction step comprises adding a quantity of the sulfide ore to the oxidized fluid mass in a separate reduction zone to accomplish a double decomposition of the oxide and the sulfide in accordance with the following reaction:



My invention further resides in conducting these two reactions, which I shall refer to hereinafter as (1) the oxidation step or reaction, and (2) the reduction step or reaction, respectively, under conditions such that the heat evolved in the exothermic oxidation step provides the heat necessary to maintain the mass in a molten condition and to supply the heat absorbed in the endothermic reduction step without input of heat from an external source.

My invention in its preferred embodiment also resides in conducting the said oxidation and reduction steps not only in sequence but also in a continuous manner, wherein there is maintained a continuous, cyclic flow of molten metal from the reduction zone to the oxidation zone, a continuous supply of molecular oxygen such as air, commercially pure oxygen, or oxygen enriched air to the oxidation zone, a continuous supply of sulfide ore to the reduction zone in substantially stoichiometric relation to the oxygen supplied to the oxidation zone so as to balance Reactions 1 and 2, a continuous removal of sulphur dioxide from the reduction zone, and a continuous recycling of molten metal from the reduction zone to the oxidation zone in quantity sufficient to maintain a mass of molten, circulating and reaction medium and to preserve continuity of the process.

Referring now more specifically to the drawings, a charge of substantially pure metallic lead 1 is initially heated until it assumes a molten form, the said preheating being accomplished by oil burners or other heating elements (not shown) which are suitably positioned to operate under closed storage tank 2 containing the lead. Also all conduits are heated by blow torch or other means. After the lead in storage tank 2 has assumed a molten form and is brought to a temperature of approximately 700° F., the oil burners or heating elements may be completely shut down as they are not needed during the subsequent operation of the continuous process for reasons which will hereinafter appear.

The molten or liquid lead, upon reaching its proper temperature, is circulated through the system by means of a conventional-type, variable speed centrifugal lead pump 4 driven by motor 5 located outside of the tank, which causes the lead to be forcefully conducted through conduit 6 and to be ultimately introduced through port 7 into oxidation chamber or zone 8. Pump 4 may, of course, be adjusted to regulate the rate of flow or circulation of the lead through the system. Simultaneously with the introduction of the molten lead through port 7, molecular oxygen, such as air, oxygen, or oxygen enriched air, from a compressory source (not shown) is introduced through conduit 9 and port 10 into com-

bustion chamber 8. The molten lead introduced through port 7 and the oxidizing gas introduced through port 10 are thoroughly mixed together during their turbulent travel together down and around baffles 11, which are provided around the interior walls of chamber 8. The oxygen in the gas which is introduced through port 10, upon contacting and being thoroughly mixed, as aforesaid, with the hot molten lead, chemically unites with a portion of that metal to form lead oxide, the combustion resulting in the evolution of a tremendous amount of heat:



15 The lead oxide produced as a result of the above reaction remains in molten form and it is in this way carried along by the larger molten stream of relatively pure lead, which has not chemically united with oxygen in mixing chamber 8 in its travel therethrough.

20 By employing air (in which the oxygen content is determined), or oxygen or air which has been enriched with a predetermined amount or percentage of oxygen, I am able to control the above reaction with considerable accuracy and am able to oxidize a predetermined desired fractional part of the entire quantity of the molten metal. I prefer to oxidize less than one-half of the entire metal bath in order that there is always maintained a relatively larger quantity of the original metal which serves in effect as the basic circulating medium for carrying out the process in the apparatus. Although 25 it is more or less optional with a particular operator as to what fractional part of the entire quantity of metal will be oxidized, once this factor has been decided upon, the oxidizing gas (which contains a known amount of oxygen) may be continuously introduced into the circulating metal stream substantially in proportions for a balanced equation in a reaction between the oxygen contained in the oxidizer and the predetermined fractional part of the metal to be oxidized. Determination of the proper 30 proportions for balanced equations between the various reactants used in the process may be computed according to well-known principles of chemistry and the manner of determining these factors are not, *per se*, considered as a part of this invention.

35 The molten mixture consisting of the lead and lead oxide, after passing through the oxidizing chamber is conducted through an orifice 12 into the reaction chamber or zone 13. Lead sulfide preferably in the form of ore or lead ore concentrate (PbS) is preferably fed from hopper 14 in a predetermined regulated rate of flow into reaction chamber 13 by means of a conventional type screw feeder 15. As above indicated, it is an important object and advantage of the present invention to utilize relatively high-grade commercially available lead sulfide ore and/or concentrate. Preferably, lead concentrate containing from 55% to 85% lead (63% to nearly 100% lead sulfide), such as produced commercially through beneficiation of low-grade ore by the flotation process or other processes, is employed. The term "finely-divided, relatively high-grade, undiluted lead sulfide ore" as used herein and in the claims is intended to mean either lead sulfide ore and/or lead concentrate which is predominately lead sulfide and which is fine enough to all pass through a standard No. 20 sieve, as specified in ASTM specification E11-39, which appears in 1949 ASTM

Standards, part II, "Non-Ferrous Metals," page 1016, published in 1950. The finely-divided ore or concentrate, fed into reaction chamber 13 by screw feeder 15, mixes with and chemically unites with the lead oxide carried along as a part of the molten mixture, as hereinabove described. Baffles 16, similar to baffles 11, are provided to insure a thorough mixing of the molten mass and lead sulfide together and thereby insure a more complete chemical reaction between the lead sulfide and the lead oxide. This latter chemical reaction is violent and produces metallic lead and sulfur dioxide gas as illustrated in the following chemical equation:



As above indicated, the screw feeder permits the finely-divided PbS to be fed into the reaction chamber at a predetermined regulated rate of flow. The amounts of PbS continuously introduced into the reaction chamber for reaction with the PbO should, of course, preferably be substantially in proportions for a balanced equation in a reaction between the lead sulfide contained in the ore and the lead oxide. It will be recalled that the PbO carried along in the molten stream was itself produced through controlled oxidation of a predetermined fractional part of the original metal bath, and, therefore, the total amount of PbO available for reaction with the PbS is readily ascertainable.

It is also preferable to introduce into the reaction chamber along with the lead sulfide concentrate, relatively small quantities of a suitable flux, such as limestone, lime, or soda ash, for example, which will react with contained silica impurities in the concentrate to form relatively fusible slag. Increased fusibility of the slag will, of course, minimize metal loss through its inclusion within slag ultimately removed from the bath.

Residual diluent gases from the oxidizing chamber and evolved sulphur dioxide, intermixed with hot molten metallic lead and non-gaseous impurities, leave reaction chamber 13 through discharge conduit 17 and are introduced into the vortex of a closed impellor, such as indicated at 18, which is adapted to operate within roof enclosed agitation chamber 19. Violent intermixing created by agitation of the impellor favors the completion of the reactions in the reaction chamber and the formation of a clean and fluid slag. The agitation also causes the intermixed gases to rise through the molten lead contained in chamber 19. The escape of these gases is prevented by means of a hood which covers the agitation chamber.

The impellor, heretofore indicated at 18, may be of generally conventional construction and is shown as being of a type commonly used in ore flotation process apparatus. More specifically, this type of impellor comprises a pair of oppositely disposed, spaced, circular plates 20 and 21 housing a plurality of radial fins 22. An upper tubular casing 23 defining an enlarged inlet mouth 24 in flow communication with the interior of the impellor provides an opening through which drive shaft 25, which is anchored at 26 to bottom plate 21, may project upwardly. Shaft 25, in turn, may be rotated by means of a motor 27, or other driving means, located outside of agitation chamber 19.

Rotation of the impellor will continuously centrifugally force outwardly the molten mass and contained gas introduced into mouth 24 of

the impellor from conduit 17. The impellor functions to continuously suck downwardly into agitation chamber 19 the materials from reaction chamber 13 and prevent back-pressure from building up in the system by virtue of the SO<sub>2</sub> gas produced in chamber 13. Moreover, as above suggested, the impellor creates a turbulent agitation within chamber 19 and thus serves to insure a thorough mixing and reaction between any unreacted PbO and PbS flowing from the reaction chamber 13. A suitable flue 30 supported by hood 31 conducts the gases to a point of suitable disposal. The sulfur dioxide concentration in these gases is exceptionally high, and it may therefore be inexpensively recovered for use in the manufacture of sulfuric acid, liquid sulfur dioxide, or other commercial by-products.

The agitation chamber is provided with a port 32 through which solid particles of slag may be removed from the surface of the bath at such intervals or under such conditions as this may become necessary. This port is provided with a hinged gas-tight door 33 so that under normal operating conditions no gas can escape through said port.

From the agitation chamber the liquid mixture of molten lead and molten slag together with suspended solid particles is conducted through a suitable conduit 34 into storage reservoir 2.

The lead reservoir tank 2 is a quiet zone which permits the separation by gravity of the molten lead from its molten and solid impurities. At one side of this reservoir is a lead well 35 in communication with the reservoir via opening 36 and from which molten lead may be continuously or intermittently withdrawn, as through port 37, at a rate substantially equivalent to the rate of entry into the system of the contained lead in the sulfide ore. The reservoir is likewise provided with a slag tap hole 38 through which accumulated slag may be periodically tapped from the surface of the lead. Within this reservoir and taking its feed therefrom, is variable-speed, centrifugal pump 4, heretofore designated. This pump continuously pumps molten lead to the oxidation chamber, thus closing the circuit and making this a continuous cyclic process.

As heretofore stated, it is a principal object of the present invention to teach and to provide a continuous and thermally self-sustaining cycle-process of metal reduction. In the cyclic process just described, and as stated heretofore, the exothermic oxidation reaction:



evolves sufficient excess heat to compensate for radiation and other heat losses. In the practice of the invention normal reasonable precautions should be taken in the insulation, arrangement, and type of equipment employed to prevent any undue or excess heat losses; although, on the other hand, the excess heat produced is such that no extraordinary, elaborate, or unusual precautions need be taken to maintain the necessary heat balance between the reactions sufficient to maintain a calorific self-sustaining continuous process.

Although it is not essential to use any particular type of material in constructing the instant apparatus, other than a material which can suitably withstand the various temperatures and chemical reactions taking place during the process as above enumerated, I prefer to use as my construction materials ceramic refractories for

reaction chamber linings and heavy cast iron, similar to that used in common lead refining kettles, for the reservoirs and pump parts. Not only can cast iron of this type endure the temperatures, pressures and chemical reactions produced during the process, but such material upon once being brought up to proper temperature has a marked tendency to hold and retain the heat imparted to it. This tendency is especially valuable in my process for the reason that the apparatus may be stopped or shut down for a period of several hours while retaining sufficient heat to prevent the molten lead from cooling and solidifying. Should the lead solidify in the tanks or conduits during a shut-down, it is only necessary to heat the equipment by oil burners and blow-torches, as earlier described, until the metal assumes a molten form. The pump and impellor may then be started and when the lead is freely circulating within the system, the process may be continued as before and as above described.

Although I have described the present invention in some detail for purposes of illustration and example, it is understood that various changes and modifications may be practiced within the spirit of the invention and scope of the appended claims.

I claim:

1. In a method of reducing lead from relatively high-grade undiluted lead sulfide ore, the successive steps comprising, forming a molten bath of relatively pure lead, continuously circulating said molten bath of lead from a starting point throughout a series of chambers back to said starting point, during said circulation through a first chamber introducing into said molten bath an oxidizing gas containing a known quantity of oxygen in an amount substantially less than will oxidize the entire quantity of said lead in said molten bath, whereby a molten mixture comprising predetermined amounts of molten lead and lead oxide is formed, during said continuous circulation through a second chamber introducing into said molten mixture for reaction with said lead oxide amounts of finely-divided, relatively high-grade, undiluted lead sulfide ore substantially in proportions for a balanced equation in a reaction between said predetermined amount of lead oxide and the lead sulfide contained in said ore, whereby there ensues a chemical reaction resulting in the production of a molten mixture of molten lead and sulphur dioxide gas, removing said sulphur dioxide gas from said molten mixture, and then circulating a part of said lead back to said first chamber for recirculation back through said series of chambers and removing a part of said metal for recovery.

2. A method of reducing lead from relatively high-grade undiluted sulfide ore according to claim 1 and wherein the amount of oxidizing gas introduced into the bath of molten lead is substantially less than the amount of said gas which will oxidize one-half of the entire quantity of molten lead circulating through said first chamber.

3. A method of reducing lead from relatively high-grade, undiluted lead sulfide ore according to claim 1 wherein said gas consists of relatively pure oxygen.

4. A method of reducing lead from relatively high-grade, undiluted lead sulfide ore according to claim 1 wherein said gas consists of oxygen enriched air.

5. A method of extracting lead from its sulfide which comprises; providing a mass of lead in a molten condition, providing also a mass of predominantly lead sulfide, introducing the molten lead into an oxidation zone, and also introducing in said oxidation zone an oxidizing agent in quantity sufficient to oxidize a substantial proportion of the lead to its oxide according to the exothermic reaction  $2\text{Pb} + \text{O}_2 = 2\text{PbO}$ , introducing the molten mass of lead and oxidized metal to a reduction zone; adding said lead sulfide to the molten mass in the reduction zone in quantity sufficient to reduce substantially all of the lead oxide according to the endothermic reaction  $\text{PbS} + 2\text{PbO} = 3\text{Pb} + \text{SO}_2$ ; separating sulphur dioxide from the reduced mass; and returning a sufficient quantity of molten metal from the reduction zone to the oxidation zone to maintain a body of molten, circulating and reaction medium for continued operation of the process; said quantity of oxidizing agent being sufficient to provide the heat absorbed in said endothermic reaction and to also maintain the mass in molten condition without input of heat from an external source.

6. The method of claim 5 wherein the said oxidizing agent introduced into said oxidation zone comprises molecular oxygen, and wherein the amount of lead sulfide introduced into said reduction zone is in substantially stoichiometric proportion to the quantity of molten lead oxidized in said oxidation zone for the said reaction  $\text{PbS} + 2\text{PbO} = 3\text{Pb} + \text{SO}_2$ .

7. The method of claim 5 wherein the mass of predominately lead sulfide contains from about 55% to 85% by weight of lead and which is fine enough to all pass through a standard No. 20 sieve.

8. A continuous method of extracting lead from its sulfide which comprises: providing a mass of lead in a molten condition; providing also a mass of predominantly lead sulfide; continuously circulating the molten lead into an oxidation zone, and also continuously introducing molecular oxygen into said zone in quantity sufficient to oxidize a substantial proportion of the lead to its oxide according to the exothermic reaction  $2\text{Pb} + \text{O}_2 = 2\text{PbO}$ ; continuously circulating the fluid mass of molten lead and oxidized lead to a reduction zone; continuously adding said lead sulfide to the molten mass in the reduction zone in quantity sufficient to reduce substantially all of the lead oxide according to the endothermic reaction  $\text{PbS} + 2\text{PbO} = 3\text{Pb} + \text{SO}_2$ ; continuously separating sulphur dioxide from the reduced mass; and withdrawing a portion of the lead for recovery and continuously recirculating a sufficient quantity of said lead from the reduction zone to the oxidation zone to maintain a body of molten circulating and reaction medium for continued operation of the process; said quantity of oxygen being sufficient to provide the heat absorbed in said endothermic reaction and to also maintain the mass in molten condition without input of heat from an external source.

9. The method of claim 8 wherein the amount of lead sulfide introduced into said reduction zone is in substantially stoichiometric proportion to the quantity of molten lead oxidized by said molecular oxygen in said oxidation zone for the said reaction  $\text{PbS} + 2\text{PbO} = 3\text{Pb} + \text{SO}_2$ .

10. The method of claim 8 wherein the mass of predominately lead sulfide contains from about 55% to 85% by weight of lead and which is fine

## 11

enough to all pass through a standard No. 20 sieve.

11. The method of extracting lead from its sulfide which comprises: providing a mass of predominantly lead sulfide containing not more than about 37% of impurities; providing a mass of molten lead; continuously introducing said molten lead into an oxidation zone; continuously introducing molecular oxygen into said oxidation zone in quantity sufficient to react with not more than 50% of molten lead to form a molten mass of lead and oxidized lead, continuously circulating said molten mass into a reduction zone and continuously introducing into said zone said lead sulfide in a proportion approximately stoichiometrically related to the oxygen introduced into the oxidation zone so as to approximately balance the reactions:

- (1) (exothermic)  $2\text{Pb} + \text{O}_2 \rightarrow 2\text{PbO}$   
 (2) (endothemic)  $\text{PbS} + 2\text{PbO} \rightarrow 3\text{Pb} + \text{SO}_2$

continuously removing sulfur dioxide resulting from Reaction 2; and continuously recirculating a sufficient quantity of molten lead from the reduction zone to the oxidation zone to maintain a continuous, cyclic flow of molten metal; out un-

5

10

15

20

25

## 12

der conditions to utilize the heat evolved in Reaction 1 the quantity of oxygen introduced into said oxidation zone being such that the heat generated in Reaction 1 is sufficient to supply the heat absorbed by Reaction 2 and also to maintain the mass in molten condition without input of heat from an external source.

12. The method of claim 11 wherein the mass of predominantly lead sulfide contains from about 55% to 85% by weight of lead and which is fine enough to all pass through a standard No. 20 sieve.

CHARLES B. FOSTER.

## References Cited in the file of this patent

## UNITED STATES PATENTS

| Number    | Name           | Date          |
|-----------|----------------|---------------|
| 494,349   | Rosing         | Mar. 28, 1893 |
| 543,735   | Roux           | July 30, 1895 |
| 882,193   | Francis        | Mar. 17, 1908 |
| 894,383   | Imbert         | July 28, 1908 |
| 997,405   | Mitchell       | July 11, 1911 |
| 1,938,582 | Davis          | Dec. 12, 1933 |
| 2,416,628 | Kalling et al. | Feb. 25, 1947 |